

Dec. 9, 1958

J. S. EDGAR

2,863,686

ROCK DRILL BIT

Filed April 27, 1954



# United States Patent Office

2,863,686

Patented Dec. 9, 1958

1

2,863,686

## ROCK DRILL BIT

John Stanley Edgar, Saint Catharines, Ontario, Canada, assignor to Thompson Products, Ltd., Saint Catharines, Ontario, Canada, a corporation of Ontario

Application April 27, 1954, Serial No. 425,938

2 Claims. (Cl. 287—126)

The instant invention relates to an improved drill assembly and method of producing the same, and more particularly, to an improved rock drill assembly of the type wherein the bit is detachable from the shank and is retained thereon by an interference or press-fit, and to an improved method of producing such an assembly.

Although the teachings of the present invention will be applicable to a number of phases in the drilling art, the particular invention will be described in detail in connection with rock drill bits and assemblies containing the same. Such assemblies comprise a metal drill bit body, usually made of steel, having carbide inserts mounted on the drilling face thereof and having a socket on the back thereof for receiving the shank. The shank is press-fit into the socket during assembly; and after the drill bit has been used for a while and requires repair or rebuilding, the drill bit body is forced off the shank, repair is needed, and then press-fit back onto the shank. This operation may be repeated a number of times. It has been found, however, that the life of these parts, and particularly the drill bit body, is greatly shortened because of the failure to obtain a proper fit between the bit body and the shank after a relatively few number of removals and replacements of the bit body on the shank. Damage, particularly to the walls of the bit socket, by tearing or otherwise injuring the walls, apparently during the press-fit assembly or disassembly, causes an improper fit between the two parts and thus shortens the useful life thereof.

Although certain precautions have been taken heretofore to avoid this damage, these have left much to be desired. A particular difficulty herein resides in the fact that these parts must be handled at the drilling site, where production time is of great importance and where the operators are often not cooperative in carrying out the various operational steps required to avoid damage.

The instant invention resides in the provision of a protective lining for the surfaces which are press-fit, which is substantially fool-proof in that it avoids the necessity for having complete cooperation with the mining operators in preventing damage to the parts. The instant invention provides for the use of a permanent thin crystalline coherent lubricant coating which is applied to either the walls of the shank or the walls of the socket or both, and which remains on these walls during the repeated assembly and disassembly steps so as to continuously furnish protection therefor. It has been found that this type of coating provides adequate lubrication for the assembly and disassembly steps, without interfering with proper functioning of the two parts when press-fit together, during drilling, etc.

It is therefore an important object of the instant invention to provide an improved method of preparing the same.

It is a further object of the instant invention to provide an improved drill assembly comprising a metal drill bit body having a wall portion defining a shank-receiving

2

ing socket therein, a metal shank adapted to be press-fit into said socket and having a wall portion for engaging the socket wall portion, and a thin crystalline coherent lubricant coating of a metallic salt chemically bonded to at least one of said wall portions, said bit and said shank being press-fit together; and an improved method of producing such a drill assembly which comprises the step of coating at least one of said wall portions with a chemical solution which reacts with the metal to produce thereon the thin crystalline coherent lubricant coating of a metallic salt chemically bonded thereto.

Other and further objects, features and advantages of the instant invention will become apparent to those skilled in the art from the following detailed disclosure thereof and from the drawings which form a part hereof and which describe a preferred embodiment of the instant invention.

On the drawings:

Figure 1 is a full view in elevation of a drill bit assembly embodying the instant invention;

Figure 2 is an elevational sectional view taken substantially along the line II—II of Figure 1;

Figure 3 is an exploded view with parts shown in section and parts broken away of the drill bit body and the shank of the instant assembly;

Figure 4 is an end view of the drill bit body, taken substantially along the line IV—IV of Figure 3;

Figure 5 is an enlarged fragmentary sectional view taken substantially along the line V—V of Figure 3; and

Figure 6 is a fragmentary enlarged detail view taken substantially along the line VI—VI of Figure 3.

As shown on the drawings:

In Figures 1 and 2, there is shown a drill bit assembly indicated generally by the reference numeral 10, which comprises a metal drill bit body 11 having a wall portion 11a defining a generally cylindrical (but tapering slightly inwardly) shank-receiving socket therein, a metal shank 12 adapted to be press-fit into the socket defined by the walls 11a and having a corresponding wall portion 12a for engaging the socket wall portion 11a, and a thin crystalline coherent lubricant coating 13 of a metallic salt chemically bonded to at least one of said wall portions, in this case, the socket wall portion 11a, said bit body 11 and said shank 12 being press-fit together.

In the particular bit body 11 here shown, the drilling face 11b has four generally rectangular grooves 11c extending radially from a central aperture, at 14 (designated in Figure 2) and the grooves 11c seat suitable carbide inserts 15a, 15b, 15c, and 15d therein (the inserts being shown in full view in Figure 2). The inserts 15 provide the necessary cutting edges for effecting the drilling; and the bit body 11 is grooved at 16a, 16b, 16c and 16d, on the drilling face 11b between the inserts 15a, 15b, 15c and 15d so as to provide a fluid outlet for drilling fluid which passes downwardly through the central aperture 14 then radially outwardly through channels at 17 on the drilling face 11b and then longitudinally back or upwardly through channels designated 18. The shank 12 is also apertured at 19 with an axially aligned channel 20 which provides for the flow of drilling fluid downwardly the full length of the shank 12 into the drill bit socket defined by the walls 11a (the space S in the socket not occupied by the shank 12, if any appreciable space is present, also being filled with drilling fluid) and on downwardly through the axially aligned aperture 14 in the bit body 11. The details of structure outlined in the instant paragraph are merely exemplary of a type of drill bit assembly which may be used in the practice of the instant invention; and it will be appreciated that various other drill bit body structures may also be used as well as various other shank structures, the essence of the present in-

vention residing in the positioning of the lining 13 in the drill bit socket.

Referring to the lining 13 shown in Figure 2, it will be noted that this lining or coating 13 is applied only to the walls 11a of the drill bit body, but it will be appreciated that the lining or coating may be applied to both the walls 11a and the walls 12a (as is shown in Figure 3) or it may be applied only to the walls 12a of the shank 12. This latter structure, although operative for the purposes of the instant invention, is less preferred, because the shanks are often made at drilling site where the coating might be more difficult to apply, whereas the bit bodies are manufactured in a shop whereat the application of the coating would be less difficult. For this reason, the most preferred embodiment of the invention is one wherein the walls 11a defining the drill bit socket have the coating 13 applied thereto, with a corresponding coating optionally applied to the shank 12.

Referring now to Figures 3, 4, 5 and 6, it will be noted that the general structure of the drill bit assembly shown therein is substantially identical to that shown in Figures 1 and 2, with the single exception that a coating or lining such as the coating 13 is applied to both the socket (designated by the reference numeral 23a) and the shank (whereat it is designated by the reference numeral 23b). The reference numerals used in Figures 3, 4, 5 and 6 in the "20" series of numbers indicate the parts or elements which are the same as those designated by the corresponding number in the "10" series of numbers used in Figures 1 and 2; in other words, the drill bit body 21 of Figures 3, 4, 5 and 6 is the same as the drill bit body 11 of Figures 1 and 2, etc. It will also be noted that the coatings 13, 23a and 23b are shown without section lines for the sake of simplicity in Figures 2, 3 and 4; and are shown in section in the enlarged views of Figures 5 and 6.

The present invention is based upon the discovery that the particular coatings here employed possess a certain combination of properties which include self-lubrication to an extent sufficient to protect the metal parts but to an extent insufficient to cause slipping between the metal parts during the drilling operation or other breakdown of the interference fit therebetween. In addition, the instant coatings have sufficient adherence to the surface to which they are applied to permit repeated use of the parts thus coated without breakdown of the coating layer. This provides the unique advantage of having the protective layer already installed in, for example, the drill bit body 11 so that operators in the field are not required to take any steps at all in connection with applying a protective coating or otherwise attempting to accomplish this purpose. The necessity for complete cooperation between the drill operators and the bit manufacturers in connection with taking the necessary precautionary steps is eliminated.

The instant coatings are of a type known as surface conversion or chemical dip coatings, which are produced by actually converting the surface of a metal into an oxide, salt or other chemical compound of exceedingly low solubility in the environment to which the metal surface is ultimately to be exposed. In a sense, these coatings may be considered to be corrosion-resistant and are applied to the surface of the metal so as to provide a coating of the corrosion product of the metal, which prevents further corrosion. In general, these surface films or coatings are formed from phosphate, chromate or oxalate solutions. The most preferred being phosphate solutions, which are applied in the so-called "Parkerizing" process, and related processes involving improvements thereover. Some of the earlier phosphate coatings applied to ferrous surfaces were applied by the use of a solution of phosphoric acid and ferrous sulfate. Zinc sulfate may be substituted for the ferrous sulfate in applying suitable coatings. The original "Parkerizing" process, however, involved the use of primary man-

ganous phosphate in aqueous solution. The processes of this type, including the "Parkerizing" process and the improvements made thereon are well known to the art and the specific details thereof need not be described herein. It will be noted, however, that each of these processes, which produces a thin crystalline coherent lubricant coating of a metallic oxide or salt on the metal surface, which crystalline coating is chemically as well as physically bonded to the metal surface, may be used in the practice of the instant invention. The crystals of these coatings are in heterogeneous crystalline joint with the metal base and are tightly grown together with the latter.

At the present time, a number of commercial processes are employed for the purpose of applying coatings, which have now been found to be unusually satisfactory for use in the instant invention. A typical example of a coating formulation which has been found to give particularly satisfactory results in the practice of the invention is as follows:

| Ingredient:                    | Parts |
|--------------------------------|-------|
| Zinc oxide-----                | 250   |
| Sodium nitrate-----            | 600   |
| Nitric acid 42° Bé-----        | 750   |
| Zinc dihydrogen phosphate----- | 900   |
| Water -----                    | 2500  |

Using 70 pounds of the foregoing solution in 750 pounds of water, a properly diluted solution is obtained. This formulation is disclosed in Glasson Patent No. 2,296,844, issued September 29, 1942. The instant formulation is applied by immersing the shank or the drill bit body of the instant invention in the solution for from 1 to 5 minutes at temperatures within the range of 160-200° F. Other procedures may, of course, be employed. Such other procedures include the use of different times and temperatures, the times and temperatures being correlated merely to the extent necessary to apply an appreciable amount of the instant crystalline coating. Any appreciable amount of the instant coating, which skilled operators can readily detect, is sufficient to afford the advantages of the instant invention, so the particular details relating to the amount of coating applied are those operating conditions which suit the particular skilled operator in the art. For example, in the original "Parkerizing" process, times of as much as 3 to 4 hours were used, although modern methods have now improved this process to the extent that coating times of as little as 30 seconds may be used. The solution may employ other dihydrogen phosphates in place of the above recited zinc dihydrogen phosphate, such as the corresponding salts of cadmium, calcium, strontium, barium, chromium, and manganese. A small amount of a copper salt in the bath also tends to reduce the processing time, but the alkali nitrate here used is generally considered superior for this purpose.

Other operative coatings may also be applied from chromic acid, dichromate or strong alkali solutions. It will also be appreciated that the application of these coatings is not necessarily limited to ferrous metals, although in the drill bit art the bit body or matrix is almost invariably made of steel.

The coatings thus produced on the metal surfaces are preferably deposited from aqueous solutions of reagents capable of producing such coatings, which may be the salts of the same metal which forms the surface of the article or salts of a metal different from that of the article, or mixtures of such salts. With ferrous metals, coatings of iron phosphates and/or complexes thereof are preferred. Corresponding salts of oxalic acid may also be used. The films or coatings thus formed are dense thin coherent coatings which are crystalline in character wherein the acid has combined both chemically and physically with the metal of the base.

Processwise, the invention consists in producing a drill bit assembly 10 which comprises forming a metal drill

bit body 11 having a wall portion 11a defining a shank-receiving socket therein, forming a metal shank 12 adapted to press-fit into the socket and having a wall portion 12a for engaging the socket wall portion 11a, coating at least one of the wall portions 11a and 12a with a chemical solution (i. e., a phosphate solution) which reacts with the (ferrous) metal to produce thereon a thin crystalline coherent lubricant coating of a metal salt (i. e., an iron phosphate salt or complex) chemically bonded to the wall portion (in this case the wall 11a), and press-fitting the shank 12 into the socket.

The instant invention has been field tested and the tests have clearly demonstrated the superior results obtained in the practice of the instant invention.

It will be understood that modifications and variations 15 may be effected without departing from the scope of the novel concepts of the present invention.

I claim as my invention:

1. A drill assembly comprising a metal drill bit body having a wall portion defining a shank-receiving socket 20 therein, a metal shank press-fit into said socket and having a wall portion engaging the socket wall portion, and a thin crystalline coherent lubricant coating of a metallic

5  
10

phosphate salt chemically bonded to at least one of said wall portions in the area of engagement therebetween.

2. A method of producing a drill assembly, that comprises providing a steel drill bit body having a wall portion defining a shank-receiving socket therein, providing a steel shank adapted to be press-fit into said socket and having a wall portion for engaging the socket wall portion, coating at least one of said wall portions with a dilute phosphate solution which reacts with the steel to produce thereon a thin crystalline coherent lubricant coating of a metallic phosphate salt chemically bonded thereto, and press-fitting said shank into said socket.

References Cited in the file of this patent

UNITED STATES PATENTS

|           |         |       |              |
|-----------|---------|-------|--------------|
| 803,911   | Leyner  | ----- | Nov. 7, 1905 |
| 2,015,727 | Prey    | ----- | Oct. 1, 1935 |
| 2,042,088 | Bedford | ----- | May 26, 1936 |
| 2,274,961 | Horger  | ----- | Mar. 3, 1942 |

FOREIGN PATENTS

|         |               |       |                |
|---------|---------------|-------|----------------|
| 5,778   | Great Britain | ----- | 1908           |
| 803,911 | Great Britain | ----- | Sept. 20, 1939 |